

# United States Patent [19]

Davis et al.

[11] 3,867,155

[45] Feb. 18, 1975

[54] SMOKELESS EXOTHERMIC HOT TOPPING COMPOSITIONS

[75] Inventors: James A. Davis, Worthington; Arthur R. Elsea, Columbus, both of Ohio

[73] Assignee: Consolidated Ceramic Products, Inc., Blanchester, Ohio

[22] Filed: Oct. 31, 1973

[21] Appl. No.: 411,401

[52] U.S. Cl..... 106/38.27, 164/53, 249/202, 249/DIG. 5

[51] Int. Cl..... B28b 7/36

[58] Field of Search..... 106/38.27; 164/53; 249/202, DIG. 5

[56] References Cited

UNITED STATES PATENTS

3,025,153 3/1962 Cross ..... 164/53 X

|           |        |                  |           |
|-----------|--------|------------------|-----------|
| 3,144,690 | 8/1964 | Ruckingham ..... | 164/53 X  |
| 3,325,316 | 6/1967 | MacDonald .....  | 164/53 X  |
| 3,713,852 | 1/1973 | Wiley .....      | 106/38.27 |

Primary Examiner—Lewis T. Jacobs

Attorney, Agent, or Firm—Wood, Herron & Evans

[57]

## ABSTRACT

Smokeless exothermic hot topping compositions are provided for application to the metal hot top of a cast ingot or a casting riser to improve the yield of usable metal or inhibit piping. Exothermic compositions containing aluminum, iron oxide and inert filler materials are disclosed which produce no visible smoke when used as hot topping materials.

23 Claims, No Drawings

## SMOKELESS EXOTHERMIC HOT TOPPING COMPOSITIONS

### BACKGROUND OF THE INVENTION

Exothermic ingot-topping materials have been used for many years to improve the yield of usable material from killed-steel ingots. The topping materials normally are used in conjunction with hot top insulating boards or casings mounted at the top of an ingot casting mold. Hot top boards or casings usually insulate the top 1 1/2 to 2 feet of the cast ingot sides; and exothermic materials are added to the top of the cast metal to provide heat and insulate the metal surface. Hot top boards and exothermic topping materials together maintain a reservoir of molten metal to feed the shrinkage normally encountered in the center of a solidifying ingot top. This shrinkage is a phenomenon commonly called "piping" and, therefore, exothermic compositions are sometimes referred to in the art as "anti-piping" compositions. During subsequent rolling, the top or riser portion of the metal ingot is sheared off and discarded and the balance of the ingot is processed into the desired shapes.

Most known ingredients used in exothermic materials include oxidizers, fuels, inert ingredients, and fluxes. Oxidizers include mill scale ( $Fe_3O_4$ ), iron ore ( $Fe_2O_3$ ), alkali metal nitrates, manganese or chromium oxide (or other metal oxides), metal chlorates or picrates; fuels include aluminum, ferrosilicon, titanium, magnesium, silicon or alloys thereof, carbon (in the form of coke, charcoal, coal, charred oat hulls, etc.), organic compounds (resin binders), and the like; inert ingredients include sand, grog, slags, clay binders, alumina cement, perlite, vermiculite, or the like; and fluxes include sodium chloride, fluorides such as calcium fluoride or sodium fluoride. Representative prior art patents which disclose such compositions include British Pat. Nos. 673,605; 745,668; 769,719; 852,377; 870,668; 969,311; Canadian Pat. No. 631,077; U.S. Pat. Nos. 2,514,793; 2,791,816; 2,850,373; 2,937,425; 3,025,153; 3,104,996; 3,132,061; 3,183,562; 3,198,640; 3,347,721; and 3,672,918.

Conventional exothermic topping compositions produce considerable smoke and fume during use. Foundry workers are subjected to risky working conditions and health hazards caused by such smoke. Federal and state statutes have been enacted which require safer and healthier working conditions in plants and foundries. Attempts have been made in the past to overcome the hazards of smoke and fume caused by exothermic topping materials. For example, it has been proposed in U.S. Pat. No. 3,713,852 that smoke evolution can be minimized in certain exothermic compositions by critically controlling particle sizes of specific oxidizers and fuels and maintaining the ingredients of such compositions within specified compositional limits. Another proposal has been to employ organic additives to consume fumes produced by certain exothermic compositions as illustrated by U.S. Pat. No. 3,728,102. There is still however a critical need for an exothermic topping composition which is smokeless and which still provides other essential functional requirements.

### SUMMARY OF THE INVENTION

This invention is directed to an exothermic hot top-

ping composition for use in the primary production or casting of metal, particularly iron or steel. Exothermic compositions have been discovered which are completely smokeless and provide adequate feeding of an ingot hot top or cast metal riser. In fact, actual production runs for ingot steel castings have demonstrated that exothermic compositions of this invention perform without producing any visible smoke. In contrast, known exothermic hot topping materials produce considerable smoke.

This invention is predicated in part upon the discovery that certain oxidizer, fuel and inert filler materials can be proportioned to provide smokeless exothermic compositions. In a preferred form, the compositions contain mill scale ( $Fe_3O_4$ ), aluminum and inert filler materials. These compositions contain an effective amount of an oxide of iron up to about 50% by weight and an effective amount of fuel of aluminum or aluminum alloy providing up to about 15% by weight aluminum and the balance being predominantly composed of inert filler materials. These components are proportioned to provide smokeless compositions. "Smokeless" as the term is broadly used herein to characterize compositions of this invention means no visible smoke or only trace amounts of visible smoke. However, compositions are advantageously provided as mentioned above in accord with the principles of this invention which produce no visible smoke. Smokeless as it applies to compositions of this invention can also be equated herein to a Ringelmann number less than 1 or equivalent opacity of less than 20%.

Generally, smoke is considered to consist of the gaseous products of burning organic materials, such as wood, coal, or tobacco, rendered visible by the presence of small particles of carbon, which finally settle as soot. However, in the field of physical chemistry, any suspension of solid particles in a gas is termed smoke. Sometimes, however, the term "smoke" is used to include fume, vapor, or dust that resembles smoke. In this application, the term smoke will include the latter meanings. The Ringelmann Smoke Chart and equivalent opacity is used herein to read visible emissions of smoke. The Ringelmann Chart was developed by Maximilian Ringelmann in the late 1800's and has been a useful tool ever since, at least in controlling visible emissions, which constitutes the nuisance form of air pollution. The Ringelmann Chart is thoroughly covered in the Bureau of Mines Information Circular No. 8333 (May, 1967), and this Circular is incorporated herein by reference to ascertain smoke emissions by Ringelmann number and opacity. Another article incorporated herein by reference is "Reading Visible Emission" by Jerome J. Rom, U.S. Department of Health, Education and Welfare, April 1968. The Ringelmann system is virtually a scheme whereby graduated shades of gray, varying by five equal steps between white and black, may be accurately reproduced by means of a rectangular grill of black lines of definite width and spacing on a white background. The rule by which charts may be reproduced is as follows:

Card 0 — All white.

Card 1 — Black lines 1 mm thick, 10 mm apart, leaving white spaces 9 mm square.

Card 2 — Lines 2.3 mm thick, spaces 7.7 mm square.

Card 3 — Lines 3.7 mm thick, spaces 6.3 mm square.

Card 4 — Lines 5.5 mm thick, spaces 4.5 mm square.

Card 5 — All black.

The chart, as distributed by the Bureau of Mines, provides the shades of cards 1, 2, 3, and 4 on a single sheet, which are known as Ringelmann No. 1, 2, 3, and 4, respectively. To use the chart, it is supported on a level with the eye, at such distance from the observer that the lines on the chart merge into shades of gray, and as nearly as possible in line with a smoke source. The observer glances from the smoke, as it issues from the smoke source, to the chart and notes the number of the chart most nearly corresponding with the shade of the smoke, then records this number with the time of observation. A clear source is recorded as No. 0, and 100 percent black smoke as No. 5. Although the Ringelmann Chart is only useful in evaluating black or gray emissions, a principle of equivalent opacity was developed which makes possible the application of the Ringelmann principle to other colors of smoke. Opacity simply means the degree to which transmitted light is obscured. Below is the relationship between Ringelmann number and opacity:

| Ringelmann No. | Opacity % |
|----------------|-----------|
| 1              | 20        |
| 2              | 40        |
| 3              | 60        |
| 4              | 80        |
| 5              | 100       |

Preferred operable ranges of main components are about 25-45% of an oxide of iron, about 9-13% aluminum fuel as aluminum metal or alloys thereof with the balance of predominantly inert materials. These main components are finely divided to permit blending for uniformity of reaction. However, the mesh sizes of iron oxide, aluminum and inert fillers can vary over wide ranges as the examples demonstrate to achieve smokeless compositions and, therefore, mesh sizes of these components are not critically limiting upon the principles of this invention. In another of its aspects, a minor amount of granular graphite can be incorporated in the exothermic composition to provide an early ignition of the exothermic reaction without deleteriously affecting its smokelessness. An amount of graphite on the order of about 1 to about 4% by weight has been found to fulfill these purposes when employed in the compositions of this invention.

The inert filler materials are selected from a class of diverse materials, particularly refractory materials in granular form such as fire clay, fire-clay grog, bauxite, olivine, perlite, expanded perlite, silica flour, silica sand and the like. The mesh size of such inert filler materials can vary over considerable ranges. It is preferred, however, to use coarse mesh sizes whose average mesh size is within the range of about -12 to about +100 to insure smokelessness. Finer particles have a tendency to cause melting or higher reaction temperatures of the exothermic compositions in use which in turn has been found to induce the formation of smoke. The mesh sizes for inert materials, however, can be varied within the essential compositional parameters of this invention as will be appreciated by the working examples and description of this invention.

An additional advantage is secured by the compositions of this invention when an insulating slag forming material is included with the main components. The inert filler material can also function as an insulating slag forming material. In a preferred form, about

5-15% by weight of expanded perlite is used as a slag forming additive which provides an insulating property to the compositions in use. Also, it is desirable to include binders which permit pelletization of the exothermic compositions to reduce dust formation. Binders such as fire clay are employed to assist in pelletization.

In accord with one best mode of operation, an exothermic hot topping material that is completely smokeless is provided according to the principles of this invention when that composition consists essentially of about 35-42% by weight mill scale, 11-13% by weight of aluminum, 30% by weight raw fire clay, about 10% by weight expanded perlite, about 5% by weight fire-clay grog and about 3% by weight graphite. This composition is especially preferred in preparing pelletized materials as just mentioned in accordance with the above procedures. Each of the ingredients performs certain functions. The mill scale ( $Fe_3O_4$ ) provides the oxygen for the combustion of fuel, that is, the aluminum and the graphite. The expanded perlite serves to slow down the reaction and also acts as an insulator to help retain most of the heat in the steel ingot material. The fire clay is added as a binder to permit pelletizing of the damp mixture and the fire-clay grog is added as a compatible inert ingredient. The perlite, fire clay and fire-clay grog all act as inert ingredients that decrease the reaction rate and help retain the evolved heat in the steel ingot by their insulating properties in the slag. Of course, when granular materials are desired rather than the pelletized form, the compositional content of the inert refractory materials can be varied as the examples below demonstrate. For example, if pelletization is unnecessary to reduce dust, the fire clay could be replaced with other materials that would improve the ignition characteristics of the mixture and the insulating properties of the resulting slag. Again, pelletization has the advantage of eliminating dust and may be particularly suited where it is important to reduce the amounts of dust as well as reduction of smoke or fumes.

A main finding in practicing this invention is the control of the compositional limits both of iron oxide oxidizer and aluminum fuels below certain critical amounts. An operable exothermic amount of oxide of iron up to about 50% by weight and aluminum fuel up to about 15% by weight has been found essential in providing smokelessness. The ratios of oxidizer and fuel will vary within these ranges of amounts. A stoichiometric ratio of about 3.2 to 1 of iron oxide to aluminum fuel is satisfactory, however, it is not critically essential to a practice of this invention. It has been discovered that amounts of iron oxide can be increased within the specified compositional range provided the aluminum fuel is decreased to achieve a smokeless composition. For example, as the amount of iron oxide is increased above about 40% towards about 50% by weight, the aluminum fuel should be decreased from about 15% by weight towards about 10% by weight to achieve smokelessness. These and other variations of the parameters of this invention will be further understood by reference to the examples which follow.

#### EXAMPLES 1-11

Exothermic hot topping compositions of this invention were prepared as 1000-gram samples in Examples 1-11 containing ingredients in weight percent as listed in Table I as follows. All compositions of Table I additionally contained 30% raw fire clay, except Examples

5 and 6 in which 27% raw fire clay was used. These compositions were ignited on 100-pound induction-furnace heats of carbon steel maintained at about 2900°-3000°F by supplying a small amount of power to the induction coil.

All samples were prepared in the form of  $\frac{1}{4}$ -inch or small pellets. The mill scale ( $\text{Fe}_3\text{O}_4$ ) was first screened through a  $\frac{1}{2}$ -inch-mesh screen, heated to about 650°F to dry and degrease it, pulverized in a ball mill, and screened through a 20-mesh screen. The ball mill used for pulverizing the mill scale was 20 inches in diameter and was loaded about half full with 2-inch-diameter steel balls. The mill scale was ground for 15 to 20 minutes. The aluminum metal (grindings and turnings) was screened through a 1/2-inch-mesh screen to remove trash, heated to about 450°F to dry and degrease it, pulverized in the same ball mill for 20 to 30 minutes, and screened through a 12-mesh screen. The prepared aluminum and mill scale for each sample were ball milled together for 3 to 5 minutes, primarily to achieve thorough mixing. Other ingredients were added to the mill scale and aluminum without any prior preparation. Alsifer (alloy of about 20% Al, 40% Si and 40% Fe) of about -100 mesh, expanded perlite of about -10 mesh, raw fire clay of about -12 mesh, fire-clay grog of about -12 mesh and graphite of about -12 mesh were used where indicated in Table I. The compositions thus prepared were pelletized by rolling the damp mixtures in a small cement mixer. The densities of the pelletized mixtures of Examples 3-5 and 8-11 were about 39-43 pounds/cubic foot and Examples 6-7 were about 83-86 pounds/cubic foot. The  $\frac{1}{4}$ -inch or smaller pellets were then tested for their properties as exothermic hot topping compositions and the results are reported in Table I.

15

cases, only a trace of smoke or no smoke was observed during the performance of the compositions in Examples 1-11. By the term "trace" of smoke it is meant that only an insignificant amount of smoke was noted in 5 these examples, i.e., much less smoke than was produced by the bare steel surface by comparison. Such a trace corresponds to a smoke rating considerably less than Ringelmann No. 1 or approximately 5% opacity. No visible smoke at all was observed during the testing 10 of Example 3 and Examples 6-9. Of Examples 1-11, Example 3 was considered to be the best from the standpoint of no visible smoke being produced and, from a standpoint of overall performance of reaction time and temperature.

6

#### EXAMPLE 12

A 100-pound sample of an exothermic hot topping composition was prepared in accordance with the composition of Example 3 reported above employing the same ingredients. For this purpose, 40 pounds of mill scale, 12 pounds of aluminum, 30 pounds raw fire clay, 10 pounds of expanded perlite, 5 pounds of fire-clay grog and 3 pounds of graphite were weighed. These components were mixed in a small cement mixer while about 6.5% by weight water was added very slowly. The total mixing time was approximately 30 minutes. Afterwards, the damp mixture was screened through a  $\frac{1}{2}$ -inch-mesh screen to break up any large pellets and then dried at 350°F. The dried, partially pelletized mixture was packaged in 10-pound lots in polyethylene bags.

The material of Example 12 was evaluated on commercial steel ingots having a hot top cross sectional area of approximately 24 inches square. The hot top-

TABLE I

| Example Number | Mill Scale | Aluminum Grindings | Alsifer | Ex-panded Perlite | Fire-Clay Grog | Graphite | Reac-tion Time | Reaction Temp. °F | Slag Condition | Smoke |
|----------------|------------|--------------------|---------|-------------------|----------------|----------|----------------|-------------------|----------------|-------|
| 1              | 45         | 12                 | —       | 10                | 3              | —        | 4'30"          | 2750              | Gummy          | Trace |
| 2              | 45         | 12                 | —       | 10                | —              | 3        | 6'35"          | 3000              | Gummy          | Trace |
| 3              | 40         | 12                 | —       | 10                | 5              | 3        | 8'20"          | 3000              | Gummy          | None  |
| 4              | 40         | 12                 | —       | 10                | 8              | —        | 7'40"          | 3160              | Gummy          | Trace |
| 5              | 45         | 7                  | 8       | 10                | —              | 3        | 9'15"          | 2800              | Gummy          | Trace |
| 6              | 45         | 7                  | 8       | —                 | 10             | 3        | 8'0 "          | 3060              | Gummy          | Trace |
| 7              | 45         | 7                  | 8       | —                 | 10             | —        | 7'30"          | 2550              | Gummy          | None  |
| 8              | 40         | 7                  | 8       | 10                | 2              | 3        | 8'30"          | 2650              | Gummy          | None  |
| 9              | 40         | 7                  | 8       | 10                | 5              | —        | 8'0 "          | 2550              | Gummy          | None  |
| 10             | 40         | 8                  | 8       | 10                | —              | 4        | 8'45"          | 2600              | Gummy          | Trace |
| 11             | 40         | 12                 | —       | 10                | 3              | 5        | 8'0 "          | 3150              | Gummy          | Trace |

The reaction time reported in Table I was that time required for the 1000-gram sample to react completely. The maximum temperature produced by the reacting exothermic composition is reported as measured with an optical pyrometer with no correction for emissivity (the true temperatures would be higher than reported in Table I). The topping compositions of Examples 1-11 did not melt in usage upon being ignited on the steel heats but did appear to become Gummy. In all

60 ping material was used in conjunction with insulating boards of a type commonly employed for commercial operations. One commercial ingot was topped with approximately 20 pounds of the above formula while another ingot was topped with approximately 30 pounds of the above formula by placing two and three bags respectively of 10-pound lots of the formula employed in this example. In both the commercial ingots, the exothermic hot topping material of this example did not

produce any visible smoke. Furthermore, the exothermic hot topping composition performed satisfactorily as an ingot hot topping material.

#### EXAMPLES 13-20

Compositions containing mill scale, aluminum and fire clay in varying percentages by weight were formulated as listed in Table II. In Examples 13-20, the mill scale particle sizes were of about -2+10 mesh and the aluminum particle sizes were about -10+30 mesh. The fire clay particle sizes were approximately -12 mesh. In other words, the mill scale particle sizes were such that the particles passed through a 2 mesh screen and were retained on a 10 mesh screen, whereas the aluminum particles passed through a 10 mesh screen and were retained on a 30 mesh screen. The ingredients for each of the Examples 13-20 were thoroughly mixed together and then the granular 1000-gram mixtures of each Example were spread onto 100-pound molten steel heats having a temperature of about 2900°-3000°F as in Examples 1-11. Again, the exotherm of the topping material was measured with an optical pyrometer without correction for emissivity and the results are reported in Table II.

TABLE II

| Ex. No. | Mill Scale | Alumi-num | Fire Clay | Reaction Temp. °F | Observation               |
|---------|------------|-----------|-----------|-------------------|---------------------------|
| 13      | 30         | 10        | 60        | 2140              | No visible smoke          |
| 14      | 30         | 15        | 55        | 2600              | No visible smoke          |
| 15      | 40         | 10        | 50        | 2400              | No visible smoke          |
| 16      | 40         | 15        | 45        | 3100              | Trace of smoke            |
| 17      | 50         | 10        | 40        | 3000              | Faint trace of smoke      |
| 18      | 10         | 20        | 70        | —                 | No reaction in 15 minutes |
| 19      | 10         | 15        | 75        | —                 | No reaction in 15 minutes |
| 20      | 10         | 10        | 80        | —                 | No reaction in 15 minutes |

Table II demonstrates that when the mill scale was varied between 30% and 50% by weight with the aluminum varying between about 10-15% by weight, an exothermic reaction was observed between about 2100°-3100°F. In the case of Examples 13-15, no visible smoke was observed. A trace or a faint trace of smoke was observed in Examples 16-17, respectively, but such an amount was less than the bare surface of the metal itself. Furthermore, in connection with Examples 16-17, the negligible amounts of smoke were comparable to the trace amounts of the preceding examples.

In the case of Examples 18-20, wherein the mill scale was present in an amount of about 10% by weight with the aluminum varying between about 10-20% by weight, no reaction was observed within 15 minutes of the test. Accordingly, these examples demonstrate that in accordance with the principles of this invention exothermic smokeless hot topping compositions are provided when the amount of an oxide of iron (mill scale) is within the range of about 25-50% by weight and the aluminum is in the range of about 9-15% by weight in the presence of a granular inert refractory material. Within such proportions, exothermic hot topping materials are prepared which perform in a satisfactory manner and which will not smoke or only negligible amounts of smoke considerably less than a Ringelmann

satisfactory manner and which will not smoke or only negligible amounts of smoke considerably less than a Ringelmann No. No. 1 rating are observed. By comparison of Examples 13-17, as the amount of mill scale is increased from above about 40% by weight to about 50% by weight, the amount of aluminum is reduced from about 15% by weight to completely eliminate visible smoke. These examples also demonstrate that the mesh sizes of mill scale and iron oxide may be varied, by comparison with Examples 1-11, and the objectives of the invention are still achieved.

#### EXAMPLES 21-27

For purposes of comparison with preceding examples, particularly Examples 13-20, Examples 21-27 were performed. Compositions containing mill scale, aluminum and fire clay in varying percentages by weight as indicated in Table III were prepared as above. However, in Examples 21-27, 80% of the mill scale particle sizes were about -10+50 mesh and the balance was approximately 70% of about -10+150 mesh and 30% of about -150 mesh. The aluminum particle sizes of Examples 21-27 comprised 85% of about -30+100 mesh with the balance of 15% being approximately -12+30 mesh. All the test runs in this series were made by placing the exothermic hot topping material on molten steel as in Examples 13-20 above and the temperatures of the reactions recorded by an optical pyrometer as above. The results are reported in Table III as follows.

TABLE III

| Ex. No. | Mill Scale | Alumi-num | Fire Clay | Reaction Temp. °F | Observation               |
|---------|------------|-----------|-----------|-------------------|---------------------------|
| 21      | 30         | 15        | 55        | 2160              | No visible smoke          |
| 22      | 40         | 10        | 50        | 2120              | No visible smoke          |
| 23      | 40         | 15        | 45        | 2250              | No visible smoke          |
| 24      | 50         | 10        | 40        | 2900              | No visible smoke          |
| 25      | 30         | 5         | 65        | —                 | No reaction in 15 minutes |
| 26      | 40         | 5         | 55        | —                 | No reaction in 15 minutes |
| 27      | 10         | 20        | 70        | —                 | No reaction in 15 minutes |

Examples 21-24 demonstrated that exothermic hot topping compositions of this invention exhibit no visible smoke while providing an exothermic reaction. Furthermore, particle sizes of oxidizer and fuel are not critically important to the principles of this invention as demonstrated by comparison of the particle sizes of the ingredients in Table III with Tables I-II. In connection with Examples 25-27 no reaction was observed within 15 minutes of the test. Thus, this series of comparative examples 21-27 reconfirmed that there is an amount of mill scale within the range of about 25-50% that can be combined with an amount of aluminum between 10-15% by weight to provide the satisfactory results.

#### EXAMPLE 28

A composition in granular form was prepared and tested according to the procedures of Examples 21-27 except that the formula comprised the following ingredients:

40% mill scale  
12% aluminum

30%  
10%  
5%  
3%

-Continued  
raw fire clay  
expanded perlite  
fire-clay grog  
graphite

Furthermore, the mesh size of the mill scale in this example was about -150 mesh and the aluminum mesh size was about -150. Example 28 had a reaction temperature of about 3200°F and only a trace of smoke was observed comparable to the trace amounts of the preceding examples. This example thus further illustrated that other mesh sizes other than those reported above are suitable for use according to the principles of this invention.

#### EXAMPLE 29

The procedures of Example 28 were repeated except that a mesh size for the aluminum was about -30+150, in other words the aluminum particles passed through a 30 mesh screen and were retained on a 150 mesh screen. The hot topping composition of Example 29 had a reaction temperature of about 2950°F and exhibited a faint trace of smoke comparable to the trace amounts of the preceding examples. This example further illustrates the wide latitude of mesh sizes for the oxidizer and the fuel for use in the hot topping compositions of this invention to achieve smokelessness.

#### EXAMPLES 30-40

This series of exothermic hot topping compositions with varying amounts of ingredients were prepared in accordance with the techniques described in Examples 1-11 except that the compositions of Examples 30-40 were in mixed granular form and not pelletized. These exothermic compositions as detailed in Table IV hereinafter were ignited on 100-pound, induction-furnace steel heats in accordance with the procedures of Examples 1-11 and the results reported in Table IV.

on the metal top than the pelletized mixtures used in Examples 1-11. Eliminating the pelletizing step however tends to increase the dust created when the exothermic hot topping compound was handled. Examples

5 30-33 also employed the addition of iron oxide ( $Fe_2O_3$ ) for part or all of the mill scale ( $Fe_3O_4$ ). These examples also demonstrate that  $Fe_2O_3$  may be substituted for the mill scale ( $Fe_3O_4$ ) with equivalent results. The  $Fe_2O_3$  used in these experiments was pulverized pure  $Fe_2O_3$  10 having a mesh size of approximately -200.

Examples 34-40 were conducted for the purpose of varying the amounts of mill scale and aluminum fuel with varying proportions of raw fire clay, calcined fire clay, bauxite, or olivine. The raw fire clay and bauxite

15 were calcined before use. The olivine was about -100 mesh and composed of magnesium silicate and 7% iron silicate. The bauxite contained about 88% alumina and was about -16+80 mesh. As observed by Examples 32-40, various inert filler materials can be used with

20 the oxidizer and fuel. Further, the granular nature of the slag reaction product can be enhanced by substituting higher melting refractory inert materials where a granular, chunky or crusty slag reaction product is desired for more easy removal from the hot metal top.

25

#### EXAMPLES 41-48

For the purpose of demonstrating that the mesh size of the inert filler material in the exothermic composition can have an effect on the smokelessness of an exothermic composition, Examples 41-48 were performed on an experimental basis. In the case of these examples, 30 200-gram samples of ingredients listed in Table V were prepared in the form of  $\frac{1}{2}$  to  $\frac{3}{4}$  inch pellets in a manner similar to that described above. The mill scale and aluminum were of the same mesh as used in the Examples 1-11. The ignition time was measured in minutes and seconds required for the 200-gram sample to ignite in a clay-graphite crucible heated to about 2100°F. The reaction time was recorded in minutes and seconds as

TABLE IV

| Ex. No. | Mill Scale | Alumi-nium | Expanded Perlite | Graphite | Raw Fire Clay | Other                            | Reaction Time Minutes | Max Reaction Temp. °F | Slag Condition | Smoke | Remarks        |
|---------|------------|------------|------------------|----------|---------------|----------------------------------|-----------------------|-----------------------|----------------|-------|----------------|
| 30      | 30         | 12         | 10               | 3        | 30            | 10 $Fe_2O_3$<br>5 fire-clay grog | 15                    | 2400                  | Gummy          | None  | Some dust      |
| 31      | 20         | 12         | 10               | 3        | 30            | 20 $Fe_2O_3$<br>5 fire-clay grog | 16                    | 2400                  | Gummy          | None  | Some dust      |
| 32      | —          | 12         | 10               | 3        | 30            | 40 $Fe_2O_3$<br>5 fire-clay grog | 9                     | 3000                  | Crusty         | Trace | Some dust      |
| 33      | —          | 12         | 10               | 3        | 30            | 36 $Fe_2O_3$<br>9 fire-clay grog | 10                    | 2600                  | Crusty         | None  | Trace of dust  |
| 34      | 40         | 12         | 10               | 3        | 10            | 25 fire-clay grog                | 6                     | 3200                  | Chunky         | Trace | Trace of dust  |
| 35      | 40         | 12         | 10               | 3        | —             | 35 fire-clay grog                | 8                     | 3100                  | Chunky         | Trace | Trace of dust  |
| 36      | 40         | 12         | —                | 3        | —             | 45 olivine                       | 7                     | 3000                  | Crusty         | Trace | Few sparks     |
| 37      | 30         | 14         | —                | 3        | —             | 53 olivine                       | 11 1/2                | 3200                  | Crusty         | Trace | Few sparks     |
| 38      | 30         | 14         | —                | 3        | —             | 53 bauxite                       | 9                     | 3200                  | Chunky         | Trace | Slag was       |
| 39      | 30         | 14         | —                | 3        | 53            | —                                | 11                    | 2600                  | Chunky         | None  | crumbly under- |
| 40      | 30         | 14         | 10               | 3        | 43            | —                                | 15 1/2                | 2540                  | Chunky         | None  | neath          |

Examples 30-40 demonstrated the applicability of the principles of the invention to granular exothermic mixtures. These granular mixtures are more spreadable

65 required for the 200-gram sample to complete the reaction. The reaction temperature produced by the reacting exothermic materials at the start and the maximum

temperature achieved was measured with an optical pyrometer with no correction for emissivity. In the case of Examples 41 and 45-46, the coarse raw perlite used was about -6+35 mesh whereas the fine raw perlite in Example 42 was ball milled to about -100 mesh. The bauxite used in the examples was aluminum ore composed of impure hydrated aluminum oxide. In Example 43, the fine bauxite was approximately -200 mesh, whereas the coarse bauxite in the remaining Examples 44 and 47-48 was about -16+80 mesh. The results of these examples appear in Table V.

parative test sample was placed upon a molten steel heat in accordance with the procedures of Examples 21-24. The reaction time was approximately 1 1/2 minutes and a maximum temperature of greater than 3400°F was measured. The composition of this test sample produced a considerable amount of smoke on an order of magnitude greater than Ringelmann No. 1, i.e., about 2 or more. This test sample demonstrates that as the amount of oxidizer is increased above 50% to 60% by weight with an amount of aluminum of about 16% by weight, considerable smoke is produced.

TABLE V

| Example Number | Mill Scale | Alumi-<br>num | Raw fire<br>Clay | Other | Ignition Time        | Reaction Time | Reaction Temp. °F |      | Slag Condition | Smoke      |      |
|----------------|------------|---------------|------------------|-------|----------------------|---------------|-------------------|------|----------------|------------|------|
|                |            |               |                  |       |                      |               | Start             | Max  |                |            |      |
| 41             | 30         | 15            | 30               | 25    | Raw Perlite (coarse) | 3'0"          | 3'30"             | 2200 | 2250           | Not Melted | None |
| 42             | 30         | 15            | 30               | 25    | Raw Perlite (fine)   | 2'35"         | 4'0"              | 2450 | >3400          | Melted     | Much |
| 43             | 40         | 15            | 30               | 15    | Bauxite (fine)       | 4'10"         | 4'10"             | 2250 | 3350           | Melted     | Some |
| 44             | 30         | 15            | 30               | 25    | Bauxite (coarse)     | 2'45"         | 5'0"              | 2150 | 2450           | Not Melted | None |
| 45             | 40         | 16            | 30               | 14    | Raw Perlite (coarse) | 3'0"          | 3'30"             | 2200 | 3200           | Melted     | Much |
| 46             | 40         | 17            | 30               | 13    | Raw Perlite (coarse) | 3'30"         | 2'45"             | 2200 | >3400          | Melted     | Much |
| 47             | 40         | 16            | 30               | 14    | Bauxite (coarse)     | 2'40"         | 0'45"             | —    | >3400          | Melted     | Much |
| 48             | 40         | 20            | 30               | 10    | Bauxite (coarse)     | 2'15"         | 0'40"             | —    | >3400          | Melted     | Much |

A comparison of Examples 41 and 42 reveal that the composition containing coarse raw perlite (-6+35 mesh) of Example 41 did not melt or smoke. In contrast, Example 42 containing the fine perlite of approximately -100 mesh did melt and smoke under the experimental test. Furthermore, however, as the amount of aluminum was increased above about 15% by weight to 16-17% by weight (Examples 45-46), even though the mesh size of the raw perlite was coarse, the topping material melted and much smoke was produced. The smoke produced would correspond to a Ringelmann number of greater than 1, i.e. about 2 or more. This data demonstrated that for certain compositions it is desirable to employ a coarser inert granular material and to maintain the level of aluminum fuel up to about 15% by weight to avoid smoking of the exothermic hot topping compositions.

Quite similarly, where the bauxite was of a finer mesh in Example 43, the topping material smoked considerably under the conditions of test, whereas in Example 44, the coarser bauxite did not smoke. Further, in Examples 47-48, even though the bauxite was of a coarser grain size (-16+80 mesh) with increasing amounts of aluminum from about 16 to 20% by weight in the presence of 40% mill scale the hot topping material developed considerable smoke and melted. The Ringelmann number smoke rating for Examples 47-48 was greater than 1, i.e., about 2 or more.

#### COMPARATIVE TEST

For purposes of comparison with Examples 21-24 above, a test sample of exothermic hot topping material was formulated employing the same ingredients as the mentioned examples with the same particle sizes, except that in this comparative test sample, 60% by weight of mill scale was combined with 16% by weight of aluminum and 24% by weight of fire clay. This com-

Thus, in accord with the principles of this invention the compositional relationship of both the iron oxide and aluminum fuel must be maintained below certain levels to achieve smokelessness, or a smoke rating of less than Ringelmann No. 1 or about 5% opacity. Further, complete elimination of visible smoke can be achieved in exothermic compositions where the amounts of oxide or iron and aluminum fuel are controlled in exothermically effective amounts as described above and exemplified. It has also been found that alkali nitrates, alkali or alkaline earth metal fluorides, chlorates, or chlorides tend to induce the production of smoke and noxious gasses. Only very minor amounts of such ingredients or similar ingredients can be tolerated in the compositions of this invention because of our findings in order to achieve smokelessness in accord with this invention. It has been further found that amounts of other oxidizers, particularly heavy metal oxides such as manganese dioxide, and other fuels or ingredients can be tolerated in the exothermic compositions of this invention and the advantages of this invention can be secured. Such variations in view of the teachings herein are within the scope hereof.

In view of the above examples and description of this invention, other modifications of this invention will become apparent to one of ordinary skill in the art without avoiding the spirit and scope of this invention.

#### What is claimed is:

1. A smokeless exothermic hot topping composition consisting essentially of  
an effective exothermic amount of an oxide of iron in finely divided form up to about 50% by weight, an effective exothermic amount of fuel in finely divided form selected from the group consisting of aluminum and alloys thereof, said amount providing up to about 15% by weight aluminum, with the

proviso that as the amount of iron oxide is increased above about 40% by weight towards about 50% by weight said amount of provided aluminum is decreased towards about 10% by weight and when about 50% by weight of iron oxide is reached then the amount of aluminum is no more than about 10% by weight, and the balance being predominantly composed of inert finely divided filler material, said oxide, fuel and inert material components proportioned to provide said smokeless composition.

2. The composition of claim 1 which produces no visible smoke during reaction upon the surface of molten metal.

3. The composition of claim 1 which has a Ringelmann number smoke rating of less than one.

4. The composition of claim 2 wherein said metal is iron or steel.

5. The composition of claim 1 wherein said oxide of iron is present in an amount of about 25% to about 45% by weight and said fuel is present in an amount to provide about 9% to about 13% by weight aluminum.

6. The composition of claim 5 wherein granular graphite is present in an amount of about 1-4% by weight.

7. The composition of claim 5 wherein said inert material contains an insulating refractory material.

8. The composition of claim 7 wherein said insulating material is expanded perlite.

9. The composition of claim 8 wherein said perlite is present in an amount of about 5% to about 15% by weight.

10. The composition of claim 1 as a hot topping for iron or steel.

11. The composition of claim 1 wherein said filler material is a refractory material.

12. The composition of claim 11 wherein said refractory material is selected from the group consisting of raw fire clay, silica flour, silica sand, fire-clay grog, perlite, expanded perlite, olivine, and bauxite.

13. The composition of claim 1 wherein said inert filler material has an average grain size of about -12 to about +100 mesh.

14. A smokeless exothermic hot topping composition for iron or steel consisting essentially of

about 25% to about 45% by weight finely divided mill scale,

about 9% to about 13% by weight finely divided aluminum, and

the balance being predominantly composed of inert refractory material, said mill scale, aluminum and refractory material components proportioned to provide said smokeless composition.

15. The composition of claim 14 which contains about 1% to about 4% by weight of graphite.

16. The composition of claim 14 which contains about 5% to about 15% perlite.

17. The composition of claim 14 which contains about 40% mill scale and about 12% aluminum.

18. The composition of claim 14 which produces no visible smoke during reaction upon the surface of a molten metal.

19. A smokeless exothermic hot topping composition for iron or steel having a Ringelmann number smoke rating of less than one which consists essentially of about 35-42% mill scale, about 11-13% aluminum, about 1-4% graphite and the balance inert refractory material.

20. The composition of claim 19 wherein the inert refractory material contains about 5-15% by weight expanded refractory material.

21. The composition of claim 19 wherein said ingredients are granular and homogeneously mixed together.

22. The composition of claim 20 wherein a refractory binder is present to bind said ingredients in pellet form.

23. The composition of claim 22 wherein said binder is fire clay.

\* \* \* \* \*

UNITED STATES PATENT OFFICE  
CERTIFICATE OF CORRECTION

PATENT NO. 3,867,155

DATED February 18, 1975

INVENTOR(S) James A. Davis and Arthur R. Elsea

It is certified that error appears in the above-identified patent and that said Letters Patent are hereby corrected as shown below:

Col. 1 Line 40 "969,311" should be --969,331--

Signed and sealed this 27th day of May 1975.

(SEAL)

Attest:

RUTH C. MASON  
Attesting Officer

C. MARSHALL DANN  
Commissioner of Patents  
and Trademarks